

# United States Patent Office.

LORENZO SIBERT, OF STAUNTON, VIRGINIA.

*Letters Patent No. 100,937, dated March 15, 1870.*

## IMPROVED METALLIC ALLOY TO IMITATE THE PRECIOUS METALS.

The Schedule referred to in these Letters Patent and making part of the same.

*To all whom it may concern :*

Be it known that I, LORENZO SIBERT, of Staunton, in Augusta county, and State of Virginia, have discovered a new and useful "Alloy," which may be used as a substitute for the precious metals; and I do hereby declare that the following is a full, clear, and exact description thereof.

My alloy is composed of manganic steel, copper, zinc, and manganese, in about the proportions and under the treatment hereinafter specified.

To produce an alloy representing gold, I use one part of manganic steel, three-fourths part of copper, five-eighths part of zinc, and five-eighths part of powdered manganese.

To resemble silver, I take one part of manganic steel, one-sixteenth part of copper, seven-eighths part of zinc, and one-half part of powdered manganese.

Representations of other metals may be produced by varying the proportions. These alloys are not affected by the action of acids. The first mentioned is very malleable, whilst the other is best adapted for casting, and in their higher grades are susceptible of being tempered like steel for edge-tools and other purposes for which the latter is applicable.

Common steel or iron first alloyed with manganese may be used instead of manganic steel.

In compounding, I take the molten iron or steel from the reducing-furnace into a receiver, and then mix in the copper, zinc, and manganese, keeping it well agitated. Silica may be used either in the reduction of the ore or in the receiver. Any of the carbonates, borax, or nitrate of potassa may be used as a flux.

I do not confine myself to the precise proportions above specified, although I find them to produce good results, yet they may be varied without materially changing the properties of the alloy.

Having thus described my invention,

What I claim, and desire to secure by Letters Patent, is—

An alloy, consisting of steel or iron, copper, zinc, and manganese, substantially as and for the purposes specified.

In testimony whereof I hereunto set my hand before two subscribing witnesses.

Witnesses: LORENZO SIBERT.

SYDNEY E. SMITH,  
W. MORRIS SMITH.